

1,513,815

Nov. 4, 1924.

W. R. HURD, 2ND

METAL MANUFACTURE

Filed March 11, 1918



Fig. 1.



Fig. 2.



Fig. 3.

INVENTOR.

William R. Hurd

Patented Nov. 4, 1924.

1,513,815

# UNITED STATES PATENT OFFICE.

WILLIAM R. HURD, 2ND, OF BEVERLY, MASSACHUSETTS, ASSIGNOR TO UNITED SHOE MACHINERY CORPORATION, OF PATERSON, NEW JERSEY, A CORPORATION OF NEW JERSEY.

## METAL MANUFACTURE.

Application filed March 11, 1918. Serial No. 221,812.

To all whom it may concern:

Be it known that I, WILLIAM R. HURD, 2nd, a citizen of the United States, residing at Beverly, in the county of Essex and State 5 of Massachusetts, have invented certain Improvements in Metal Manufacture, of which the following description, in connection with the accompanying drawings, is a specification, like reference characters on the drawings indicating like parts in the several 10 figures.

This invention relates to the treatment of 15 corrodible metal surfaces in the manufacture of machine parts, metal tools and the like. For the sake of illustration, the invention is herein set forth with particular reference to its applicability to the manufacture of cutters used for trimming the sole edges of shoes. It is to be understood, 20 however, that the invention is not at all limited to the treatment of edge-trimming cutters, but is applicable generally to the manufacture and reclamation of tools, machine castings and parts and various other 25 metallic articles having iron and steel or other corrodible metal surfaces.

A great deal of difficulty is experienced in 30 the preservation of such metal surfaces from corrosion which lessens their efficiency and injures their appearance. With this in view, it is one object of my invention to provide an improved method of surfacing metal articles, the practice of which will insure 35 the preservation of the articles treated not only while they are in use but when they are in storage or otherwise idle.

In addition to the general liability of 40 corrosion by exposure of machines, parts and tools to dampness and other corroding influences liable to produce rust, when they are in storage or in stock, many machines and tools, when in use, are operated only 45 intermittently with intervening periods of idleness. This is sometimes due to the fact that 50 machines or devices as a whole are operated only occasionally. In many instances, of which edge-trimming cutters furnish a good example, the particular liability to corrosion is due to the fact that the necessary equipment of a machine includes a considerable number of spare parts or interchangeable tools. For instance, edge-trimming cutters are each profiled to treat 55 sole-edges of only one style, so that the cut-

ters have to be interengaged as shoes of different styles come to the machines. The result is that although any given cutter has usually a long knife, it is subject to frequent and considerable periods of idleness. Such tools consequently are especially liable to become rusty and thus to cause 60 damage to the work operated upon.

On the other hand, it is for many uses disadvantageous to have metal surfaces too bright or highly polished. Here again the 65 use of edge-trimming cutters may be referred to as illustrative of this part of the problem. In performing an edge-trimming operation, the operator holds the shoe in his hands without any support or guide whatever, and draws its sole edge past the rapidly rotating cutter. There is nothing to control the depth of cut except the operator's judgment and skill. The reflection of 70 light from a bright cutter has a tendency to 75 dazzle the operator, making him unable to cause the trimming to extend to just the right depth. In short, either extreme in the condition of the cutter will result in unsatisfactory work.

A further difficulty met with in cutters heretofore obtainable has been that, as is very generally true of tools and machine parts, they are covered with a thick heavy oil by their manufacturer to protect them 85 from rust while in stock. It is not feasible to clean this substance all out from between the teeth before a cutter is first used, and so it greases the grinding wheel badly when the cutter is reground the first time. The 90 wheel then has to be dressed off to clean it. Moreover, the slushing of tools and machine parts by coating them with heavy oil is many times objectionable because of the liability of soiling the hands or clothing of 95 the operator or the work operated upon, this tendency being aggravated by the obvious fact that such oil-coated surfaces catch a great deal of dust and dirt.

In view of these difficulties and in accordance with a further object, my invention is directed to the protection of a metal surface with a preservative coating which is not disagreeable to the touch, is not destroyed by handling or ordinary use, and 100 will not soil the hands or clothing.

In the attainment of the above-stated and other objects, it is a particularly advanta-

geous characteristic of the invention that it provides metal surfaces liable to corrosion with a substantially indestructible dull finish, which will not require cleaning, with consequent danger of brightening. In the illustrated exemplification of the invention, the articles to be treated are immersed in a bath comprising hot paraffin and then, immediately upon removal from the bath, the 10 coated articles are subjected to an air blast to remove the surplus coating. When different sides of the articles are to be coated and the nature of the articles permits, the air jet and the coated articles are relatively 15 moved in order that the air blast may act against different sides of the articles. In the treatment of many metallic articles, it is preferable to turn or whirl the articles in the air blast, thus generating centrifugal 20 force which aids in removing the surplus coating substance. This may be effected where the articles are of such a character as to lend themselves to it by utilizing the air jet itself to whirl the articles. The surfaces of the articles hold a very thin layer 25 of coating substance effectually against removal by any ordinary handling to which the articles are subjected, and the dull character of the coating diffuses any light reflected thereby. The articles are thus preserved indefinitely in a dull, greaseless and rustless condition.

These and other aspects of the invention will be better understood from the following description of a preferred practice 35 thereof. In the drawings,

Fig. 1 represents a cutter.

Fig. 2 illustrates the roughening operation, and

Fig. 3 illustrates the step of coating the cutter.

The edge-trimming cutter illustrated in the drawings and selected for the purpose of exemplifying the invention has a depression 10 in its head, a reduced hub, as shown in Fig. 1, bored at 14, and a rib 16 to operate with the usual cutter shield or guard.

After the cutter has been formed, hardened and ground, it is preferably surface roughened. This operation may be performed in any way that will produce minute sharp edged abrasions in the surface or surfaces to be treated. The general dimensions 50 of these abrasions and of their distances from each other may well be of the same order of magnitude as the wave length of light in order to form a dull, non-reflecting surface. I perform the roughening preferably by a sand blast, as shown in Fig. 2. The apparatus there shown comprises a rotating table 18 having a number of spindles 20 on which the cutters are loosely mounted. The sand box 22 rotates above the table 18 and has a plurality of nozzles 24 through

which the sand is driven. The cutters are turned in both directions by the impact as they pass through a sand stream so that all parts of their surface are treated. Any sand blasting apparatus may be used, and the same forms no part of the present invention and need not be further described. This operation removes the scale and soda and creates a mat finish on the metal.

The cutter is then coated with an air-proof and moisture proof substance which is solid under ordinary conditions and which can be spread out in a thin coating. I have found paraffin excellent for the purpose, but I contemplate the use of other materials, for instance any waxy substances having the desired characteristics. As herein illustrated, the cutters are mounted on pins on a plate 25 (Fig. 3) arranged to rotate and to pass beneath the surface of the melted paraffin or other substance 26. The bath may be heated by flame jets 28.

In the illustrated exemplification of the method, the heat-retaining articles to be treated are heated by immersion in the hot melted coating substance to a temperature which will maintain the coating in a liquid state for a substantial period after the removal of the articles from the coating bath. After the cutters or other articles to be treated have been coated, they are removed from the bath and before the coating solidifies they are transferred from the bath to another locality where they are subjected to an air blast indicated at 30. The illustrated apparatus is so designed that the impact of the air will rotate or whirl the cutters or any other articles, provided they are rotatively mounted and have a shape that renders them responsive to the propelling force of the air. When so treated, the rotative action of the articles generates sufficient centrifugal force to aid materially in removing the surplus coating substance.

Moreover, the surplus coating substance is removed from all the treated surfaces, including a recess such as that illustrated at 10. I have found that this removes a large quantity of the coating substance which then runs back into the bath, but that the minute abrasions caused by the roughening operation retain enough of the material to make a rust-proof coating which it is very hard to remove. It appears to be actually incorporated in the finely abraded surface, being probably held by minute sharp fins struck up by the sand blast, does not rub off, and I have found that it remains unaltered after long use, and that surfaces so treated become neither polished nor rusty. The amount of the coating material remaining on the faces 32 of the teeth is so slight that it does not interfere with the operation of the grinding wheel. Moreover, metallic articles so treated are not open to the dis-

advantages, including those heretofore pointed out, arising from the slushing of the articles with heavy oil.

My invention thus provides for the manufacture of a metal surface having a permanent non-corrodible indestructible dull finish.

Having described my invention, what I claim as new and desire to secure by Letters

10 Patent of the United States is:—

1. That improvement in the art of treating metallic articles which consists in simultaneously heating and coating a metallic article by immersing it in a bath of hot melted coating substance that solidifies at ordinary atmospheric temperatures, removing said article from said coating bath, and directing an air jet against the article to remove surplus coating substance before it 15 solidifies.

2. That improvement in the art of treating metallic articles which consists in applying a coating of liquefied substance that solidifies under ordinary conditions, and removing surplus coating substance from the article by blowing against the article in such a way as to rotate the latter before the coating solidifies, thus generating centrifugal action.

30 3. The improved method of treating an article which consists in applying a coating of liquefied substance that solidifies under ordinary conditions, and simultaneously rotating the article about an axis intersecting it and blowing against the coating substance on the article.

4. That improvement in the art of treating metallic articles which consists in applying a coating of a liquefied waxy substance to an article, and removing the surplus coating substance by the conjoint effect of centrifugal force and a blast of air.

45 5. That improvement in the art of treating metallic articles which consists in coating an article with a liquefied waxy substance, and removing the surplus coating substance from the article by causing an air-blast to impinge on and rotate the article.

6. That improvement in the art of treating metallic articles which consists in im-

mersing an article in a bath of liquefied waxy substance, removing the article from said bath, and blowing against the coating substance while rotating the article so as to generate centrifugal force to remove the surplus coating substance before it solidifies.

7. That improvement in the art of treating metallic articles which consists in immersing an article in a bath comprising liquid paraffin, raising the article out of said bath, and removing surplus paraffin from the article by blowing against the liquid coating of paraffin and turning the article so as to blow against all parts of its surface.

8. That improvement in methods of treating metallic articles which consists in giving an article an excessive coating of a liquid waxy substance, and thereafter blowing against the liquid coating while relatively moving the article and the blowing means so as to remove surplus coating substance from 60 different sides of the article.

9. That improvement in methods of treating metallic articles which consists in giving an article an excessive coating of a liquid substance that will solidify at ordinary atmospheric temperatures, and thereafter simultaneously blowing against the coating and whirling the article so as to remove surplus coating substance.

10. That improvement in methods of treating metallic articles which consists in giving an article an excessive coating of a liquid substance that will solidify under ordinary conditions, and thereafter removing surplus coating substance from the article by the conjoint effect of an air-blast and centrifugal force.

11. That improvement in the art of treating metallic articles, which consists in giving an article having a recess an excessive coating of a liquid waxy substance that will solidify under ordinary conditions, and thereafter removing surplus coating substance from the recess by whirling the article and simultaneously causing a jet of air to impinge on the coating in said recess.

In testimony whereof I have signed my name to this specification.

WILLIAM R. HURD, 2ND.